

June 16, 1953

E. MARBURG

2,641,807

INGOT MOLD

Filed Dec. 6, 1950

2 Sheets-Sheet 1

*Fig. 1.*



*Fig. 2.*



*Fig. 3.*



*Fig. 4.*



INVENTOR.

Edgar Marburg  
BY  
Donald G. Dalton

HIS ATTORNEY

June 16, 1953

E. MARBURG

2,641,807

INGOT MOLD

Filed Dec. 6, 1950

2 Sheets-Sheet 2



INVENTOR.  
Edgar Marburg  
BY  
Donald G. Dalton  
HIS ATTORNEY

## UNITED STATES PATENT OFFICE

2,641,807

## INGOT MOLD

Edgar Marburg, Pittsburgh, Pa., assignor to  
 United States Steel Corporation, a corporation  
 of New Jersey

Application December 6, 1950; Serial No. 199,384

9 Claims. (Cl. 22—139)

1

This invention relates to ingot molds, especially to ingot molds of the big-end-down type and is a continuation-in-part of my copending application, Serial No. 780,055, filed October 15, 1947, now abandoned. It is preferable to use big-end-down molds if possible since it is much easier to strip the mold from the ingot and it is also possible to cast the ingot without using hot tops which may not be necessary for some types of steel. Since big-end-up ingots must project above the mold in order to be removable by a stripping crane, such ingots must always be hot-topped. However, secondary pipe was frequently found in big-end-down ingots, the type originally in almost universal use and therefore big-end-up molds were developed and came into increasing use for quality steels. However, except for steel quality, big-end-down molds are preferable to big-end-up molds from every viewpoint of steel production. The big-end-up ingot molds are more expensive than the big-end-down molds and have a shorter life. The big-end-up ingots have rounded bases and cannot stand upright in the soaking pit. They have a greater taper than big-end-down ingots and are therefore more difficult to roll. The big-end-up molds have also other disadvantages in addition to those listed above so that it is apparent that the quality advantage obtained by the use of big-end-up molds must be very important to offset the obvious disadvantages of this type of mold. The quality advantage of big-end-up molds results from the fact that the ingots are narrower at the base than at the top, which aids progressive solidification from bottom to top, thus minimizing bridging, secondary pipe and axial porosity. Even in using the big-end-up mold, however, severe axial porosity often occurs in ingots of intermediate sizes (18" to 25" wide) particularly in alloy steels. Center segregation (V-segregation) often occurs in ingots of intermediate size while outer rings of segregation (inverted V-segregation) often occur in large ingots. To reduce the occurrence of these defects, it has been proposed to increase the taper on big-end-up molds. This would reduce the occurrence of axial porosity and center segregation, but would increase inverted V-segregation. Furthermore, increased taper is undesirable because it would further enhance the difficulties of handling and rolling the ingots. Segregation defects are caused by the slow cooling of ingots cast in conventional molds. If the cooling of the ingots can be speeded up many of the defects may be minimized or eliminated.

To increase the freezing rate of ingots it has

been customary to increase the thickness of the mold wall. Besides increasing the cost and reducing the life of molds increasing the wall thickness above about 6" for intermediate sizes and 8" for large molds has other disadvantages as follows: The thick-walled molds contain more heat and must either be held out longer between use, or they will be so hot when returned for reuse as to make difficult the placing of hot tops thereon. Increasing the wall thickness has the effect of decreasing the occurrence of inverted V-segregation in ingots, but of increasing the extent and intensity of V-segregation.

I have found that if a mold is made with walls having alternate thick and thin sections around its periphery, the distance from center to center of the thin sections being not less than 12" on the internal periphery, the thick sections initially extract heat and therefore solidify the adjacent steel at a more rapid rate than do the thin sections of the mold wall. The thin sections, however, quickly heat to a higher temperature than do the thick sections so that after a period of about fifteen minutes, a considerable difference of temperature, or temperature gradient exists between the thin and thick portions of the mold. Thus heat will flow through the mold wall from the thin to the thick sections, accelerating heat extraction of the former and reducing that of the latter sections. By this means heat extraction adjacent to the thin-walled portions of the mold may be accelerated in the latter stages of solidification which is the critical time for development of V and inverted segregation. Thus the amount of V-segregation and axial porosity may be reduced in all ingots; the size of ingots free from V-segregation may be increased, while the occurrence of inverted V-segregation in ingots larger than this size may be reduced. If the molds are square or rectangular the sides are preferably made thin, so as to be at the closest distance to the center of the ingot and the corners are made thick. In round ingots, of course, no such preference exists and thin and thick sections are alternated.

It is also desirable to have the freezing rate progress from the bottom to the top and I have found that this can be done by making the ratio between the thickness of the thick and thin sections greater at the base than at the top of a big-end-down mold.

It is therefore an object of my invention to provide an ingot mold which causes ingots to freeze progressively from the bottom to the top. Another object is to provide a mold in which

2

15  
 20  
 25  
 30  
 35  
 40  
 45  
 50

55

ingots having a minimum taper ( $\frac{1}{2}$ " per side) can be cast.

Still another object is to reduce the time of complete solidification of ingots of all sizes over 18" wide.

A further object is to reduce V-segregation, axial porosity, and inverted V-segregation in commercial ingots.

These and other objects will be more apparent after referring to the following specification and attached drawings, in which:

Figure 1 is a top view of the mold;

Figure 2 is a bottom view of the mold of Figure 1;

Figure 3 is a side view of the mold in Figures 1 and 2;

Figure 4 is a side view of the mold in Figures 1 and 2 taken at right angles to Figure 3;

Figure 5 is a top plan view of a second modification of my invention;

Figure 6 is a bottom view of the mold of Figure 5;

Figure 7 is a side view of the mold of Figure 5;

Figure 8 is a sectional view taken on the line VIII—VIII of Figure 7; and

Figure 9 is a top plan view of a further modification of my invention.

The preferred embodiment of my invention is shown in Figures 1 to 4 with the thick sections being at the corners and the thin sections on the sides of the mold. As shown in Figure 1 the corner areas of the top portion of the ingot are indicated by the reference numeral 2 and extend between the dash-dot lines as indicated, while the side areas are indicated by the reference numeral 4. The corresponding corner and side areas at the bottom of the mold are indicated by the reference numerals 6 and 8, respectively.

It has been found that a convenient arrangement for varying the thickness of the walls of the ingot mold is to use the standard corrugated internal periphery as shown, while making the outer periphery of each of the sides the arc of a circle having its center outside the mold approximately on a line extending from the center of the mold through the center of the side. The outer periphery of each corner is conveniently made as the arc of a circle having its center inside the mold on a line extending through the center of the corner of the mold at approximately 45° to the adjacent sides. This arrangement gives uniform transverse cooling of the ingot. The radii of the arcs of the circles at the corners and sides as described above are determined by the thicknesses of wall desired at the center of the sides and at the corners, and by ingot sectional dimensions, in accordance with design considerations described below.

In order to vary the freezing rates to cause faster freezing at the base than at the top of the ingot, the ratio between the thickness of the corners and sides is made greater at the base than at the top of the mold. This has been conveniently done by making the lower section 1" narrower than the top section in all vertical planes. Thus, for the mold shown, the thinnest thickness of the side at the top is  $3\frac{3}{4}$ " and at the base  $2\frac{3}{4}$ ". The thickest thickness of the corner at the top is  $7\frac{3}{4}$ " and at the base  $6\frac{3}{4}$ ". Thus, the ratio of the thick corner to the thin side of the top is 2.1, while at the base the ratio is 2.5. Comparing the relative areas as indicated in the drawings, we may assume the side area to comprise 40% of the overall width and on

this basis the corner area 2 of the top is 1.37 times as great as the side area 4, while the corner area 6 of the bottom is 1.85 times as great as the side area 8. The corner-side ratio is therefore considerably greater at the bottom than at the top of the mold. With this arrangement of the mold the thickness of the side at the base is 1" narrower than the thickness of the side at the top so that the side at the base will attain a higher temperature than the side at the top. Since there is less proportional difference in thickness between corners 2 and 6 than between sides 4 and 8, and since the corners are considerably lower in temperature than the sides, considerably less difference in temperatures will occur between corners 6 and 2 than between sides 8 and 4. As a result, there will be a considerably greater temperature differential between side 8 and corner 6 at the base than between side 4 and corner 2 at the top. As a result of this increased temperature differential and the increased corner side ratio at the bottom, heat will be extracted from the sides at a considerably faster rate toward the base of the ingot than at higher levels. Also, since the wall is thinnest at the base, the actual temperatures will be maximum at the base in all vertical planes so that any heat flow longitudinally through the mold wall must be upward from the base. Thus the increased rates of transverse solidification produced by the corner/side ratio being maximum at the base cannot be interfered with by opposing heat flow in the mold wall. The above analysis of heat flow applies up to the time at which the base of the ingot becomes completely solid at which time less heat is available from the ingot interior. On account of the heat lost to the stool on which the mold rests, the base of the ingot solidifies fairly rapidly (approximately 12" high in 30 to 60 minutes, varying with the ingot size). When the temperature of the mold wall at the base drops as a result of reduced heat from the ingot, heat will flow downwardly in the mold wall, reversing the previous direction of flow. However, this will merely accelerate solidification progressively upwardly because the mold temperatures at intermediate heights prior to complete solidification will always be higher than those above until the ingot is completely solid.

Experiments have shown that a mold wall of non-uniform sections as described above, not only extracts heat from the ingot at a faster rate than attainable by a uniform mold wall of thickness equal to the thinnest part of the sides, but does so in a desirable sequence, thus resulting in the maximum improvement in the soundness of the ingot. For example, the initial rate of heat extraction by the thin sides is at the low rate normally occurring with uniform walls of the same thickness as the thinnest part of the sides. As the thin side walls become hotter, the temperature difference between them and the corners increases, resulting in increased heat flow from the sides to the corners. This rate increases until it is greatest when the mold temperature is highest. Since this requires an appreciable length of time (approximately 30 to 45 minutes), the ingot has frozen to a considerable depth before the maximum rate of heat extraction is attained. It is at this depth that inverted V-segregation normally commences to develop, but the increased rate of solidification prevents its development so that the ingot is sound with minimum segregation. In molds of uniform

## 5

wall thickness the rate of heat extraction is at a minimum when the mold temperature is greatest, because at this time there is the least difference in temperature between the ingot and mold. This is the most favorable condition for causing V-segregation in the ingot.

The mold of non-uniform wall thickness has thus been found capable of extracting heat in the critical later stages of ingot solidification at faster rates than are possible in uniform molds of any practicable wall thickness.

While Figures 1 to 4 show a preferred embodiment of my mold it is only necessary that the mold be provided with alternate thick and thin sections around its periphery with the distance from center to center of the thin sections being not less than 12" on the internal periphery of the mold. If this distance is any less, the essential temperature gradients will not develop. The ratio between the thickness of the thick and thin sections at the top compared to the thickness of the thick and thin sections at the bottom of the mold may also be increased by increasing the thickness of the corners (or thick portions) at the base while maintaining the sides (or thin portions) of the same thickness from top to bottom. Another method of varying the ratio is to maintain the same thickness of the corners and the middle of the sides vertically while reducing the diameter of the circular arc at the base and tapering it upwardly and outwardly toward the top. Still another method of varying the ratio is to decrease the thickness of the sides at the base relative to the top while maintaining the corners the same thickness throughout the height.

Another modification of my invention particularly adapted for large rectangular molds for slabbing ingots is shown in Figures 5 and 6. In these large rectangular molds (for example, 24" x 48" ingot molds), completion of the freezing of the ingot always occurs across the narrow dimension. In order to accelerate this rate of freezing, the long sides 10 are made thinner, and the ends of these long sides made thicker and/or the corners and/or the ends of the short sides 12 made thicker. As shown, the sides 10 are reduced in thickness by providing a centrally located recess 14 in the outside surface thereof. As best shown in Figures 7 and 8, this recess increases in width, but decreases in depth from the bottom upwardly until it just disappears at the top of the mold.

Increase of thickness of the side walls toward their ends for the purpose of accelerating transverse solidification across the narrow central vertical plane may also be obtained by reducing the width of the ingot toward its ends, as shown in Figure 9. In this embodiment the long sides 16 of the mold are gradually increased in width at their ends by providing a tapered inner wall 18. This method of increasing the thickness of the side walls is principally applicable to large rectangular slabbing molds, because if applied to square molds, their interiors would approach an octagonal shape. The cross-sectional shape of the ingot cast in this mold is a desirable one for rolling as it tends to prevent corner cracks which frequently develop in the initial passes in rolling. The relative thicknesses of the sides and ends of the mold at the top and bottom may be designed to insure more rapid solidification at the bottom and to prevent heat flow in the mold from top to bottom, in accordance with the principles stated hereinbefore. However, in

## 6

many instances, this variation in relative thickness of the sides and ends is not necessary in large rectangular molds.

While various embodiments of my invention have been shown and described, it will be apparent that other adaptations and modifications may be made without departing from the scope of the following claims.

I claim:

1. A rectangular ingot mold having relatively thin side walls and relatively thick end walls and corners throughout the height of the mold, the distance from center to center of the thin sides on the internal periphery being at least twelve inches, the ratio between the thickness of the end and side walls decreasing from the base to the top of the mold.
2. A rectangular ingot mold according to claim 1 in which the thickness of the side walls is reduced at the center thereof.
3. An ingot mold of generally polygonal form in cross-section having side walls and corners with at least two of the side walls being of less thickness than the adjacent corners throughout the height of the mold, the distance from center to center of the thin sides being at least twelve inches on the internal periphery, the thickness of the walls increasing from the bottom to the top thereof.
4. An ingot mold of generally polygonal form in cross-section having side walls and corners with at least two of the side walls being of less thickness than the adjacent corners throughout the height of the mold, the distance from center to center of the thin sides being at least twelve inches on the internal periphery, the ratio between the thickness of the corners and sides decreasing from the base to the top of the mold.
5. An ingot mold of generally polygonal form in cross-section having side walls and corners with the side walls being of less thickness than the adjacent corners throughout the height of the mold, the distance from center to center of the thin sides being at least twelve inches on the internal periphery, the outer periphery of each of the sides being the arc of a circle having its center outside the mold approximately on a line extending from the center of the mold through the center of the side, and the outer periphery of each corner being the arc of a circle having its center inside the mold approximately on a line extending from the center of the mold through the center of the corner, the thickness of the walls increasing from the bottom to the top thereof.
6. An ingot mold of generally polygonal form in cross-section having side walls and corners with the side walls being of less thickness than the adjacent corners throughout the height of the mold, the distance from center to center of the thin sides being at least twelve inches on the internal periphery, the outer periphery of each of the sides being the arc of a circle having its center outside the mold approximately on a line extending from the center of the mold through the center of the side, and the outer periphery of each corner being the arc of a circle having its center inside the mold approximately on a line extending from the center of the mold through the center of the corner, the ratio between the thickness of the corners and sides decreasing from the base to the top of the mold.
7. A rectangular ingot mold having relatively thin side walls and relatively thick end walls and corners, the thickness of the side walls being

reduced at the center thereof, the distance from center to center of the reduced portions of the side walls being at least twelve inches on the internal periphery, the thickness of the reduced portion of the side walls being greater at the top than at the bottom of the mold.

8. A rectangular ingot mold having relatively thin side walls and relatively thick end walls and corners throughout the height of the mold, the distance from center to center of the thin sides on the internal periphery being at least twelve inches, the ratio between the areas of the thick sections and the areas of the thin sections decreasing from the base to the top of the mold.

9. An ingot mold of generally polygonal form in cross-section having side walls and corners with at least two of the side walls being of less thickness than the adjacent corners throughout

the height of the mold, the distance from center to center of the thin sides being at least twelve inches on the internal periphery, the ratio between the areas of the thick sections and the areas of the thin sections decreasing from the base to the top of the mold.

EDGAR MARBURG.

References Cited in the file of this patent

UNITED STATES PATENTS

| Number    | Name  | Date          |
|-----------|-------|---------------|
| 1,758,823 | Blage | May 13, 1930  |
| 1,792,581 | Firth | Feb. 17, 1931 |

FOREIGN PATENTS

| Number  | Country | Date          |
|---------|---------|---------------|
| 298,717 | Germany | June 25, 1917 |